

# UNITED STATES PATENT OFFICE.

JAMES FREDERICK HOYNE, OF NEW YORK, N. Y.

## PROCESS OF MANUFACTURING FIBERLESS THREAD.

SPECIFICATION forming part of Letters Patent No. 625,033, dated May 16, 1899.

Application filed June 6, 1898. Serial No. 682,682. (Specimens.)

To all whom it may concern:

Be it known that I, JAMES FREDERICK HOYNE, a subject of the Queen of Great Britain, and a resident of the city, county, and State of New York, have invented certain new and useful Improvements in Processes of Manufacturing Fiberless Thread, of which the following is a specification.

My invention relates to the process of manufacturing fiberless thread that possesses certain properties rendering it suitable for use in the manufacture of articles as a substitute for silk or hair, which it closely resembles.

In carrying into effect said invention I dissolve purified cellulose in a basic solution of zinc nitrate, chlorid, or other suitable zinc salts of about 1.8 specific gravity at a temperature of about 90° centigrade. For some purposes I modify the result by the addition of calcium nitrate or calcium chlorid to the above solutions. I then filter the cellulose solution through felt or fine gauze to remove any suspended impurities or undissolved cellulose. The solution is then driven by pressure through small holes at a suitable temperature into methylated spirits or other liquor, which will coagulate the cellulose in the form in which it issues from the holes and at the same time wash out some of the solvent. The thread as it is formed is wound on drums, from which it is afterward unwound and the removal of the solvent completed by washing in spirits or water. The thread is then strained nearly to the breaking-point and dried in a stretched state in order to obtain the maximum strength and gloss. The thread can now or before drying be dyed and made waterproof by the usual methods and is then ready for use; but to avoid the cost of skilled manipulations involved in the ordinary processes of dyeing I add the dye and mordants in the necessary proportion to the cellulose solution before it is formed into thread. Waterproofing may in the same way be done by adding a suitable ingredient to the cellulose solution—for instance, gelatin, which is rendered insoluble in the thread in the coagulating liquor by the addition to the latter of formaldehyde or other well-known reagent.

The thread as thus formed has the property of receiving and retaining forms given to it by pressure and in this respect resembles raw silk, for which it may be substituted in various manufactures. The effect of pressure in giving the desired form is assisted by

dry or moist heat. This same property and the absence of fiber render this thread suitable for use in place of hair.

For use in the manufacture of articles usually made from dress or soft silk it is necessary to make the threads much finer than for other uses. To secure this fineness, I force the solution through very fine holes arranged in groups, using the threads from each group to form a compound thread. The twisting together of the component thread of each group is effected before or in the act of winding. After drying, however, the thread may be spun or twisted in the usual manner.

I claim—

1. The process herein described of making fiberless thread, which consists in dissolving cellulose in a basic solution of zinc salts, filtering the cellulose solution, passing the same under pressure through thread-forming medium into a coagulating compound, straining the thread and then drying the same, as set forth. 70

2. The process herein described of making fiberless thread, which consists in dissolving cellulose in a basic solution of zinc nitrate, chlorid or other zinc salts, filtering the cellulose solution, passing the same under pressure through small holes into methylated spirits, thereby coagulating the cellulose, straining the thread and drying the same while under strain, as set forth. 80

3. The process herein described of making fiberless thread, which consists in dissolving cellulose in a basic solution of zinc salts, adding dye and mordants to such solution, passing the same under pressure through thread-forming medium into a coagulating compound, then straining and drying the threads, as set forth. 90

4. The process herein described of making fiberless thread, which consists in dissolving cellulose in a basic solution of zinc salts, filtering the cellulose solution, passing the same under pressure through very fine holes into a coagulating compound, twisting together a plurality of threads, winding and stretching the same, and then drying them, as set forth. 100

Signed by me, at New York, N. Y., this 21st day of April, 1898.

JAMES FREDERICK HOYNE.

Witnesses:

JAMES M. TULLY,  
FRANK HARVEY DAVIS.